

## UNITED STATES PATENT OFFICE

2,318,544

## MANUFACTURE OF MIXED TEXTILES

Gilbert I. Thurmond and James W. Jacokes,  
Asheville, and Edward Brenner, Henderson-  
ville, N. C., assignors to American Enka Cor-  
poration, Enka, N. C., a corporation of Dela-  
ware

No Drawing. Application May 13, 1940,  
Serial No. 334,994

5 Claims.

(Cl. 18—54)

The present invention relates to the manufacture of continuous filaments, staple fiber, films and the like, and more particularly to the production of filamentous threads formed from cellulose-protein mixtures.

It is generally known at present that efforts to prepare stable cellulose-protein mixtures such as viscose-casein, have been commercially unsuccessful. In attempting to produce spinning solutions of this type, various problems have arisen causing difficulties that, up to the present, have rendered the use of the solutions impractical. Prior practice involving bringing together viscose and casein resulted in the partial precipitation of either the cellulose or protein, and if normal precautionary measures were taken to avoid such precipitation, a proper dispersion of the protein was not effected, the particles being non-uniform and heterogeneously distributed. One of the most serious drawbacks in using casein-viscose mixtures, has been that the protein content was not retained in the thread during coagulation and subsequent washing and other textile treating operations. This defeated the primary purpose of utilizing such mixtures, namely, substantial retention of the tensile strength due to the cellulose content while imparting to the thread the protein property of affinity for acid dyes similar to that of natural wool. When the protein content is removed from the thread, it lowers the tensile strength and renders it unsatisfactory from the standpoint of dyeing with wool. Heretofore, cellulose-protein threads could not, therefore, be used in combination with natural wool as the mixed fibers could not be dyed uniformly.

It is the object of the present invention to form stable cellulose-protein mixtures that can be extruded to provide a product having substantially the same strength of cellulose while exhibiting the acid-dyeing properties of proteins.

It is a further object of the invention to manufacture viscose-casein threads and the like wherein the protein content is retained during subsequent textile treating operations, or at least the protein content is controlled to impart the desired characteristics to the finished thread.

The invention further contemplates the production of continuous filaments or staple fibers which may be used alone or mixed with other fibers, particularly wool, and dyed uniformly therewith.

Another object of the invention is the provision of an improved process in which the variable factors in the spinning system are pre-

determined and adjusted in order to effect a stable viscose-casein product.

An additional object contemplates utilizing dispersing agents that will effect a uniform and homogeneous distribution of the protein and cellulose content in the spinning solution.

Other objects, such as maintaining the proper tension on the freshly formed threads during the spinning operation, controlling the composition of the coagulating bath, correspondingly adjusting the spinning conditions, etc., are comprehended by the present invention.

Referring now to the detailed process, the proper preparation of the cellulose solution and the protein solution and the mixing thereof, is highly important. Several methods which may be employed are as follows: (1) Dissolving cellulose xanthate in NaOH in the usual manner for the preparation of viscose, separately dissolving a protein such as casein, alpha protein from soy beans, zein from corn, etc., in a suitable solvent of the type KOH, NaOH, and NH<sub>4</sub>OH and then thoroughly mixing the two solutions; (2) mixing dry protein with alkali cellulose, xanthating the mixture and then dissolving the same in the normal dilute alkali employed in the preparation of viscose; (3) dissolving protein in dilute alkali, mixing the same with alkali cellulose, xanthating the mixture and then dissolving in dilute alkali; (4) dispersing dry protein in viscose; (5) mixing dry protein with cellulose xanthate and dissolving the mixture in dilute alkali; (6) mixing cellulose xanthate with a protein solution and then adding sufficient dilute alkali to dissolve the cellulose xanthate. (Where the expression "dilute alkali" is used in the preceding methods, it is intended that the aqueous solution has a concentration of less than 7% alkali, such as NaOH.)

40 The preferred method is No. 1, as it has been determined that the most homogeneous solution is prepared by utilizing the same. Either the cellulose xanthate or the protein will form a solution in dilute alkali, but when the two solutions are brought together, a solution is formed wherein some of the particles exist in colloidal suspension. In first preparing the protein solution, sufficient time must be allowed to permit the protein particles to be dissolved or uniformly dispersed and the size of the particles is preferably of the order of 1 mu or less. The time required is dependent upon the temperature, for example using casein at 20° C., 4 to 6 hours is necessary to effect a homogeneous solution or dispersion.

The time element in the dissolving, mixing and aging operations, is important because otherwise various factors impair the character of the ultimate dispersion and, therefore, detrimentally affect the spinning solution. For example, if the solution is aged too long, hydrolysis takes place. The cellulose and protein solutions should be mixed from 4 to 48 hours after the preparation of the protein solution, although satisfactory protein dispersions before mixing may be maintained for approximately 10 days. Whereas, the protein solution may be mixed into the cellulosic solution, it is preferable to mix the cellulosic solution into the protein solution. In order to obtain a thorough and uniform dispersion, a circulating pump system is suitable.

The solution is filtered either prior to, or after mixing although it is preferable to filter the solutions separately and then mix. In any case, in order to deaerate the solution, it is kept under vacuum for some time after mixing.

The mixed solution is spinnable as long as the size of the dispersed protein particles does not exceed the diameter of the normal spinneret orifices, although spinning is improved and the properties of the product are better if the size of the particles are maintained at less than 1 mu. It has been determined that more protein is washed out as the size of the particles increases.

Unless counteracted, the tendency of the protein particles is to agglomerate (in protein-viscose mixtures). The addition of proper dispersing agents to the mixture provides a more stable and homogeneous suspension that will not separate or agglomerate upon aging. In this way, the mixture may be aged or ripened to a NH<sub>4</sub>Cl index from 15 to 5, the preferred ripeness has an index of approximately 10. (The index is measured in terms of the cellulosic solution.) The dispersing agent may be added to the protein solution or the cellulosic solution or to the mixture, although it is preferably added to the protein solution. The number of dispersing agents which have been found to be particularly adaptable may be divided into two general classifications, those which are surface active and those which are non-surface active.

The surface active agents include penetrants, detergents and softeners, which will dissolve or disperse in cellulosic and/or protein solutions or their mixtures to change the interfacial tension at the cellulose-protein interface, and thereby permit a more stable dispersion. In this connection, the following groups of compounds have been found useful:

(1) *Sulfonated products of vegetable oils, fats, hydrocarbons:*

|                   |                        |
|-------------------|------------------------|
| Prestabit oil     | Sulfonated castor oil  |
| Monopol brilliant | Sulfonated olive oil   |
| Turkey red oil    | Sulfonated teaseed oil |
| Base A            | Sulfonated naphthalene |

(2) *Quaternary ammonium compounds.*—(This includes compounds which have nitrogen in the ring and compounds with nitrogen in the chain.)

|                                    |
|------------------------------------|
| Lauryl pyridinium chloride         |
| Lauryl pyridinium sulfate          |
| Stearyl pyridinium chloride        |
| Allyl pyridinium chloride          |
| Doceyl tri ethyl ammonium chloride |
| Triton S                           |
| Triton B                           |
| Triton F                           |

(3) *High molecular nitrogen bases and their salts:*

|                      |                            |
|----------------------|----------------------------|
| (a) Aliphatic nature | (b) Cyclic or heterocyclic |
| Sapamine A           | Sapamine BCH               |
| Sapamine CH          | Fixanol                    |
| Sapamine Ms          |                            |
| Sapamine FL          |                            |
| Sapamine KW          |                            |

(4) *Sulfated higher alcohols and their salts:*

|                          |                       |
|--------------------------|-----------------------|
| Tergitol penetrant 08    | Sodium oleyl sulfate  |
| Gardinol LS, and WA      | Avirol                |
| Sodium lauryl sulfate    | Tergitol penetrant 4, |
| Sodium octadecyl sulfate | and 7                 |

(5) *Amine and amide derivatives of substituted ethers and esters:*

|          |
|----------|
| Igepon A |
| Igepon T |

(6) *Sodium alkyl aryl sulfonates:*

|                |              |
|----------------|--------------|
| Nacconal NRSF  | Solvadine NC |
| Invadine B,D,N | Aresket      |
|                | Areskap      |

(7) *Sulfonated ethers:*

|            |
|------------|
| Triton 720 |
| Aerosol OT |

30 Two of the most suitable of the above noted compounds are lauryl pyridinium chloride, and Prestabit oil.

The non-surface active agents include glucose, glycerine, gelatin, gum arabic and similar types of compounds.

35 The concentration of the dispersing agent in the solution depends upon the particular agent used, the type of protein used and ratio of the cellulose-protein mixture. In general, the best results are obtained with surface active agents in a concentration of 0.01% to 1.0%. When using non-surface active agents, the preferred range is 0.1% to 3.0%.

40 If desired, a preservative may be added to the protein solution to prevent possible putrefaction due to bacterial action. Examples of satisfactory preservatives are:

|                                |
|--------------------------------|
| Dowicide B                     |
| Phenol.                        |
| Chlorinated phenol derivatives |
| Cresol                         |
| Chlorinated cresol derivatives |

45 The cellulose-protein mixed solution is spun on the same type of equipment and in a similar system as that normally used for spinning viscose thread or staple fiber. The thread may be spun with varying degrees of tension and collected on bobbins, reels, pots and the like or may be cut into staple fibers. It may then be treated for several hours in a formaldehyde solution, for example 10% formaldehyde and 10% sodium sulphate. This hardening solution reduces the solubility of the dispersed protein which, therefore, will not substantially wash out of the thread in subsequent washing, desulphurizing and other textile operations, but this naturally involves an additional expensive operation. The thread spun in this manner has a high tensile strength due to the retention of the protein content therein, and may be dyed with either direct dyes or acid wool dyes.

50 The above mentioned formaldehyde treatment may be omitted and the desired properties in the finished thread still be retained if a higher

stretch than that normally given is imparted to the thread prior to collection. In order to effect the said higher stretch, it is necessary to adjust several other factors during the spinning process. The high stretch assists in retaining the protein content in the thread provided the variable factors are adjusted accordingly. The coagulation and regeneration of the cellulose must be such that a membranous skin is formed on the surface of the individual filaments and ruptures therein are so minute that the protein will not be dissolved out.

The most important variable factor is the acid-salt ratio of the coagulating bath, although the alkalinity of the mixed solution must also be taken into consideration. Moreover, these two variables are in turn dependent on the denier of the filaments. Less important variable factors include the temperature of the coagulating bath, the maturity of the spinning solution, the spinning speed and the percentage stretch. Percentage stretch is among the less important factors only in connection with the rate of coagulation. In connection with properties affected by orientation of micelles it is very important. If the skin on the surface of the filaments can be maintained during spinning as a substantially unbroken sheath (consisting principally of cellulose), it will serve to protect the protein content from the solvent action of subsequent treating fluids. It will be readily apparent that if one variable factor is altered for spinning a particular mixed solution, the other variable factors will have to be correspondingly adjusted.

Several methods for imparting the high stretch to the thread may be utilized such as by means of two or more driven godets, or thread storage devices rotating at higher peripheral speeds and about which the thread is caused to pass a multiplicity of times. These godets or rollers may be driven in coagulating baths, heated washing baths and other treating baths; or the godets or rollers may be located alternately in and out of said baths. This system may include the so-called "two-bath system" wherein the thread is partly stretched in a coagulating bath and given an additional stretch in a hot water or hot salt solution.

It has been determined that marked losses of protein content occur in spinning high denier threads, i. e., 600/120 or 5 denier per filament. When spinning such heavier deniers without stretch, an upper critical range of acid ( $H_2SO_4$ ) concentration occurs between 9.3% and 9.7% with a fixed salt concentration. Above 9.7%, the coagulation and/or regeneration is too rapid and a major portion of the protein is dissolved out. When the same denier threads are stretched, for example from 35% to 45% during coagulation, the critical range of concentrations of  $H_2SO_4$  increases, i. e., as much as 10.5% of acid may be employed without substantial loss of the protein content.

It will be seen from the above that the cellulose-protein threads are highly sensitive to slight acid concentration variations in the coagulating bath provided the salt concentration is fixed, the theory being that high acid concentrations cause mechanical rupturing at the surface of the filaments. In which case, the protein is substantially dissolved out, thereby weakening the thread and rendering the same inert to acid wool dyes. Whereas, various ranges of acid concentrations may be employed depending on the variable factors, such ranges can be quickly determined for

each particular spinning operation. And if the coagulating bath is adjusted so that at the surface of the filaments a skin is formed during substantial stretch, a high strength cellulose-protein thread is produced that will absorb acid wool dye-stuffs in a manner comparable with that of wool-like fibers.

It is apparent that numerous suitable modifications of an operative process may be readily devised by a simple balancing of the several variables described herein as critical with respect to retention of protein in the product. In summary of the foregoing discussion it may be stated that an increase in any one of the following factors favors retention of protein:

- a.  $\frac{1}{concentration\ of\ H_2SO_4}$
- b. Concentration of salt
- c.  $\frac{1}{bath\ temperature}$
- d. Cellulose concentration
- e. Alkalinity of spinning solution
- f. Ammonium chloride index of spinning solution
- g. Take-up speed
- h.  $\frac{1}{denier}$
- i. Stretch

Given the pertinent values of an operative process, a person skilled in the art can readily devise a wide variety of other operative processes by correspondingly increasing one of the above factors to compensate for each decrease in another of them.

The ratio of the protein in the thread may vary from 0.1% to 99% based on the weight of the cellulose. However, it is usually practical to use from 15% to 35% protein.

Similarly, each of the other important factors discussed above may be varied over an extremely wide range, provided that the said factors are mutually adjusted to insure retention of the protein. For best results, it is desirable that the values of said factors be maintained in preferred ranges as defined here. Thus, the concentration of sulphuric acid in the bath is preferably within the range of 6% to 14%, while the salts may range from 12% to 30% and the bath temperature varied between 10° and 90° C. In addition to the preferred range cited above for casein concentrations it is advisable to so prepare the spinning solution that it has an alkalinity of 4% to 9% (calculated as NaOH) and an ammonium chloride index between 7 and 15. While the denier may vary from 1 to 6 per filament and the stretch imparted to the filaments be any value not substantially greater than 80%, if the other factors are suitably adjusted, it has been found preferable to maintain the linear spinning speed at a value between 50 and 80 meters per minute.

Threads formed in accordance with the above process may be given after-treatments similar to those used in the manufacture of viscose, for example they may be washed, desulphurized, bleached and dried. They are preferably bleached with a solution containing one or more bleaching agents of the type  $H_2O_2$ ,  $Na_2O_2$ ,  $Na_2BO_3$  and sulphites. The finishing treatment may also be similar to that used in the viscose process and the softening or lubricating agents to be employed depend on the particular use to which the thread is to be put.

## EXAMPLE I

36 kg. of casein are allowed to stand two hours in 108 liters of water. During this period of standing the mixture is intermittently agitated to insure complete wetting out. When the soaking is complete, 53 liters of 3.05% sodium hydroxide are added and mixed for one hour. The mixing can be effected by means of a propeller type stirrer rotating from 150 to 200 R. P. M. During this operation 1630 c. c. of Prestabot oil are added plus a small amount of phenol. At this stage, the caseinate is more fluid than viscose but is sufficiently viscous to indicate relatively slow mixing. The mixing may be carried out in alkali resistant equipment although this is not necessary as there is only about 0.5% of free sodium hydroxide. After mixing for approximately an hour, the solution should stand for 6 to 8 hours until all particles are completely dissolved.

1300 liters of normal unripened viscose (6.7% NaOH—7.9% cellulose), after having been filtered are added to the caseinate solution and thoroughly mixed. The resulting viscose-casein dispersion is of approximately the same viscosity as the viscose per se. Care must be taken during the mixing operation to prevent air from entering as much as possible, and therefore reduce the de-aeration time to a minimum. The mixed solution may be filtered if found to be necessary on microscopic examination and after ripening for approximately 18 hours to an ammonium chloride index of 10, is ready to be spun. The solution is found to have an alkalinity of 5.9% calculated as NaOH.

The viscose-protein mixture is then spun through a coagulating bath and collected at 70 meters per minute while stretching 45% between two godets.

The coagulating bath contains:

Per cent

H<sub>2</sub>SO<sub>4</sub>..... 9  
Salt calculated as Na<sub>2</sub>SO<sub>4</sub> equivalent..... 23  
Lauryl pyridinium chloride..... 0.03

The spinning bath temperature was 42° C. The thread was subsequently treated in the normal way as a continuous filament or as staple fiber.

## EXAMPLE II

53 liters of 3.05% aqueous ammonia (calculated as NH<sub>3</sub>) is added to 38 kg. of casein in 108 liters of water in which the casein has been soaked as described in Example I. The resultant mixture is agitated for one hour and 1.6 kg. of lauryl pyridinium chloride is added thereto, together with a small amount of phenol as a preservative, while the caseinate solution is agitated. Thereafter the caseinate solution is admixed with 1300 liters of viscose and after filtration, if necessary, de-aeration and ripening, is spun through a coagulating bath at 42° C. containing:

Per cent

H<sub>2</sub>SO<sub>4</sub>..... 10.0  
Salt calculated as Na<sub>2</sub>SO<sub>4</sub> equivalent..... 28.5  
Lauryl pyridinium chloride..... 0.03

and collected at 70 meters per minute while stretching 45%.

## EXAMPLE III

The spinning solution of Example I is spun through a coagulating bath at 42° C. containing

zinc sulphate to at least partially inhibit regeneration. The composition of the bath is:

|   |                                       | Per cent |
|---|---------------------------------------|----------|
| 5 | H <sub>2</sub> SO <sub>4</sub> .....  | 9.25     |
|   | Na <sub>2</sub> SO <sub>4</sub> ..... | 17.25    |
|   | MgSO <sub>4</sub> .....               | 5.0      |
|   | ZnSO <sub>4</sub> .....               | 1.0      |
|   | Lauryl pyridinium chloride.....       | 0.03     |

10 The filaments are withdrawn and passed through a bath of hot water at 75° C. while stretching 67% and collected at the rate of 70 meters per minute. The bundle of filaments may then be treated in any known manner.

15 Values of the several important variables in a number of processes found to produce casein-viscose threads are tabulated below in Table A. In this table, the column headings are similar to the reference letters given above in setting forth the tendencies toward retention, i. e., as follows:

- A. Concentration of H<sub>2</sub>SO<sub>4</sub> (percent by weight)  
B. Concentration of salt calculated as Na<sub>2</sub>SO<sub>4</sub> equivalent (percent by weight)  
C. Bath temperature (degrees centigrade)  
25 D. Cellulose concentration calculated as percent by weight of cellulose in total spinnable solids of spinning solution  
E. Alkalinity of spinning solution (percent alkali hydroxide)  
F. Ammonium chloride index of spinning solution  
G. Take-up speed (meters per minute)  
H. Denier per filament  
I. Stretch, expressed as percent

35

TABLE A

| Ex-<br>ample | A        | B        | C   | D        | E        | F    | G      | H   | I        |
|--------------|----------|----------|-----|----------|----------|------|--------|-----|----------|
| 40           | Per cent | Per cent | °C. | Per cent | Per cent |      | M.p.m. |     | Per cent |
| 1            | 10.0     | 24.0     | 43  | 75       | 5.9      | 10.0 | 71     | 5   | 45       |
| 2            | 7.0      | 22.0     | 43  | 75       | 5.9      | 10.0 | 71     | 3   | 0        |
| 3            | 9.5      | 24.0     | 50  | 80       | 5.9      | 12.0 | 71     | 2   | 35       |
| 4            | 9.0      | 24.0     | 40  | 75       | 5.9      | 10.0 | 80     | 3   | 25       |
| 5            | 9.0      | 24.0     | 20  | 80       | 5.9      | 12.0 | 70     | 3   | 45       |
| 6            | 6.0      | 20.0     | 45  | 75       | 5.9      | 11.0 | 70     | 1.5 | 15       |
| 7            | 8.0      | 24.0     | 40  | 75       | 5.0      | 10.0 | 70     | 2.0 | 35       |
| 8            | 6.0      | 26.0     | 45  | 85       | 5.0      | 12.0 | 70     | 3   | 45       |
| 9            | 10.0     | 30.0     | 40  | 75       | 6.0      | 12.0 | 75     | 1.5 | 45       |
| 10           | 8.0      | 28.0     | 50  | 75       | 6.0      | 12.0 | 70     | 1.0 | 0        |

50 The following Table B shows the characteristics of processes in which material amounts of casein were lost from the thread.

TABLE B

| Ex-<br>ample | A        | B        | C   | D        | E        | F    | G      | H | I        |
|--------------|----------|----------|-----|----------|----------|------|--------|---|----------|
| 55           | Per cent | Per cent | °C. | Per cent | Per cent |      | M.p.m. |   | Per cent |
| 1            | 10.0     | 20.0     | 20  | 75       | 5.9      | 8.0  | 60     | 5 | 0        |
| 2            | 11.6     | 23.0     | 40  | 75       | 5.0      | 10.0 | 70     | 3 | 10       |
| 3            | 10.8     | 21.0     | 43  | 75       | 6.0      | 9.0  | 65     | 5 | 0        |
| 4            | 9.8      | 21.0     | 40  | 75       | 5.5      | 10.0 | 40     | 5 | 10       |
| 5            | 12.0     | 22.0     | 50  | 70       | 6.0      | 9.0  | 50     | 4 | 20       |
| 6            | 11.0     | 22.0     | 70  | 65       | 5.0      | 10.0 | 55     | 5 | 25       |
| 7            | 10.5     | 21.0     | 45  | 75       | 5.5      | 6.0  | 70     | 5 | 15       |
| 8            | 10.0     | 20.0     | 30  | 70       | 5.5      | 8.0  | 60     | 4 | 10       |
| 9            | 9.6      | 20.0     | 25  | 70       | 5.0      | 7.0  | 75     | 6 | 0        |
| 10           | 12.5     | 22.0     | 45  | 75       | 6.0      | 7.5  | 50     | 6 | 10       |

65 What is claimed is:

1. A process for the manufacture of threads, staple fiber, films and the like from cellulose-protein mixtures which comprises mixing a viscose solution with an alkaline protein solution, adding a dispensing agent to effect a stable mixture containing highly dispersed particles of less than 10 μ, extruding the mixture into a coagulating bath containing 9 to 10% sulphuric acid and 23

70

to 30% salts of the class consisting of sodium sulphate, magnesium sulphate and zinc sulphate (calculated as sodium sulphate equivalent), to effect the formation of a skin on the formed product during subsequent stretching and then stretching the product at least 25% and after-treating the same whereby the protein content is substantially retained therein.

2. A process for the manufacture of threads, staple fiber, films and the like from cellulose-protein mixtures which comprises mixing a viscose solution with an alkaline protein solution, adding a dispersing agent to effect a stable mixture containing highly dispersed particles of less than 10 mu, extruding the mixture into a coagulating bath having a temperature of about 42° C., and containing 9 to 10% sulphuric acid and 23 to 30% salts of the class consisting of sodium sulphate, magnesium sulphate and zinc sulphate (calculated as sodium sulphate equivalent), to effect the formation of a skin on the formed product during subsequent stretching and then stretching the product at least 25%, aftertreating the same and collecting at about 70 meters per minute whereby the protein content is substantially retained therein.

3. A process for the manufacture of threads, staple fiber and the like containing characterizing amounts of cellulose and protein from cellulose-protein mixtures which comprises substantially the following steps: mixing 36 kg. of casein dissolved in an aqueous solution of sodium hydroxide with 1300 liters of viscose solution containing 7.9% cellulose, effecting a stable mixture containing highly dispersed particles having an alkalinity of 5.9% calculated as NaOH, aging the solution for approximately 18 hours to an ammonium chloride index of 10, extruding the solution into a coagulating bath having a temperature of 42° C., and containing 9% sulphuric acid and 23% salt (calculated as sodium sulphate equivalent) withdrawing and stretching the co-

agulated material 45% and collecting the same at a speed of 70 meters per minute.

4. A process for the manufacture of threads, staple fiber and the like containing characterizing amounts of cellulose and protein from cellulose-protein mixtures which comprises substantially the following steps: mixing 36 kg. of casein dissolved in an aqueous solution of ammonium hydroxide with 1300 liters of viscose solution containing 7.9% cellulose, effecting a stable mixture containing highly dispersed particles having an alkalinity of 5.9% calculated NaOH, aging the solution for approximately 18 hours to an ammonium chloride index of 10, extruding the solution into a coagulating bath having a temperature of 42° C., containing 10.0% sulphuric acid and 28.5% salts (calculated as sodium sulphate equivalent) withdrawing and stretching the coagulated material 45% and collecting the same at a speed of 70 meters per minute.

5. A process for the manufacture of threads, staple fiber and the like containing characterizing amounts of cellulose and protein from cellulose-protein mixtures which comprises substantially the following steps: mixing 36 kg. of casein dissolved in an aqueous solution of sodium hydroxide with 1300 liters of viscose solution containing 7.9% cellulose, effecting a stable mixture containing highly dispersed particles having an alkalinity of 5.9% calculated as NaOH, aging the solution for approximately 18 hours to an ammonium chloride index of 10, extruding the solution into a coagulating bath having a temperature of 42° C., and containing 9.25% sulphuric acid, 17.25% sodium sulphate, 5% magnesium sulphate, 1% zinc sulphate, withdrawing and stretching the coagulated material 67% in a bath of hot water at a temperature of about 75° C. and collecting the same at a speed of 70 meters per minute.

GILBERT I. THURMOND.  
JAMES W. JACOKES.  
EDWARD BRENNER.

CERTIFICATE OF CORRECTION.

Patent No. 2,318,544.

May 4, 1943.

GILBERT I. THURMOND, ET AL.

It is hereby certified that error appears in the printed specification of the above numbered patent requiring correction as follows: Page 4, second column, line 72, claim 1, for "dispensing" read --dispersing--; and that the said Letters Patent should be read with this correction therein that the same may conform to the record of the case in the Patent Office.

Signed and sealed this 8th day of June, A. D. 1943.

Henry Van Arsdale,

Acting Commissioner of Patents.

(Seal)